

# UNITED STATES PATENT OFFICE.

MARI E. WOLVEKAMP, OF OAKLAND, CALIFORNIA.

## COLLOIDAL COMPOUND OF ANTIMONY SULPHIDE.

1,412,438.

Specification of Letters Patent. Patented Apr. 11, 1922.

No Drawing.

Application filed May 1, 1920. Serial No. 378,230.

To all whom it may concern:

Be it known that I, MARI E. WOLVEKAMP, a subject of the Queen of the Netherlands, and a resident of the city of Oakland, in the 5 county of Alameda and State of California, have invented certain new and useful Colloidal Compounds of Antimony Sulphide, of which the following is a specification.

My invention relates to the soluble stable 10 combinations of the colloidal antimony sulphides with a protective colloidal salt, more particularly those protective colloid salts known as protalbinates and lysalbinates, which are obtained from serum 15 albumin, egg albumin or casein, for medical purposes, and my invention also relates to the process of manufacturing these products herein described and claimed.

The foremost object of my invention is to 20 provide colloidal antimony sulphides which will be stable enough to allow of their solutions being sterilized by boiling and which may be obtained as dry solids without dialyzing.

25 As a protective colloid the sodium salt of a protalbinic or a lysalbinic acid was found very suitable.

Heretofore there have been no suitable 30 colloidal preparations of these sulphides which could be transported in the dry form and which could be readily redissolved.

F. L. Usher (see reference in Chem. Abstr. Am. Chem. Soc., p. 3271, 1919) found solutions of the sulphide 1:500 very stable in 35 combination with gum arabic, but states that Paal's protalbic acid method is inapplicable to antimony compounds.

Sir Leonard Rogers (see Lancet p. 505, 1919) uses for intravenous injections in 40 kala-azar dilute and previously dialyzed solutions of antimonious sulphide in combination with gum arabic.

Whereas antimony is highly toxic to trypanosomes and tartar emetic is said to be 45 specific as a treatment for Leishmaniosis of children, readily soluble colloidal antimonious sulphide is in a very suitable form for therapeutic experimentation on such diseases.

50 In veterinary practice sodium sulphantimonate or Schlippe's salt is extensively used and a colloidal antimony pentasulphide without the useless or even harmful sodium sulphide is now rendered available by my 55 invention as a suitable compound for similar cases.

A neutral solution of colloidal antimonious sulphide in combination with sodium protalbinate is not stable in the presence of an electrolyte and the precipitation not containing a protective colloid is changed into insoluble antimonious sulphide.

By precipitating an alkaline solution of antimonious sulphide in combination with sodium protalbinate by addition of an excess 60 of an acid and washing the precipitate, the combination of antimonious sulphide and protalbinic acid will readily redissolve with an alkaline solution and form a neutral stable solution.

70 The colors of the hydrosols of the sulphides of antimony are orange-red, whereas the precipitates containing protalbinic acid are orange-yellow in color.

In the following examples there is taken 75 for each 100 grams of sodium protalbinate (obtained from serum albumin) one-fifth gram-molecule of tartar emetic for making colloidal antimonious sulphide and one-fifth gram-molecule of Schlippe's salt for making 80 colloidal antimony pentasulphide.

Example 1: Colloidal antimonious sulphide. Dissolve 100 parts by weight of sodium protalbinate and then add a colorless solution containing 64.6 parts by weight of 85 tartar emetic and 46.8 parts by weight of sodium sulphide and next add 1000 parts by volume of 2N. sulphuric acid, filter, wash the precipitate and redissolve with 1500 parts by volume of 0.1N. sodium hydroxide 90 and finally evaporate at 100° C. Yield: 103.2 parts by weight of colloidal combination containing 32.6% antimonious sulphide.

Example 2: Colloidal antimony pentasulphide. Dissolve 100 parts by weight of sodium protalbinate and then add a solution containing 96.0 parts by weight of Schlippe's salt and next add 1000 parts by volume of 2N. sulphuric acid, filter, wash the precipitate and redissolve with 2000 parts by volume 95 of 0.1N. sodium hydroxide and finally evaporate at 100° C. Yield: 110 parts by weight 100 of colloidal combination containing 36.4% antimony pentasulphide.

If instead of the 2N. sulphuric acid, there 105 is added a solution containing 21.9 parts by weight of hydrochloric acid and next added to this solution three times its volume denatured alcohol and the precipitate dried, a yield is obtained of 75 parts by weight of 110 colloidal combination containing according to analysis 51.4% antimony pentasulphide.

While the preparative methods for the production of the above named colloidal compounds are those of a generally accepted form, it is obvious that modifications and changes can be made without departing from the spirit of the invention or the scope of the claims.

I claim:

1. The soluble combination of a colloidal sulphide of antimony with a protective salt of a protein.
2. The soluble combination of colloidal antimonious sulphide with a protective salt of a protein.

3. The soluble combination of a colloidal sulphide of antimony with sodium protalbinate.

4. The soluble combination of colloidal antimonious sulphide with sodium protalbinate.

5. The combination of a colloidal sulphide of antimony with sodium protalbinate obtained from serum.

6. The combination of colloidal antimonious sulphide with sodium protalbinate obtained from serum.

20

25

MARI E. WOLVEKAMP.